# EUROPEAN PATENT SPECIFICATION

(11) **EP 3 553 197 B1**
(45) Date of publication and mention of the grant of the patent: **30.09.2020**
(21) Application number: 17878243.9
(22) Date of filing: 29.11.2017
(51) Int. Cl.: C22C 38/38, C22C 38/02, C22C 38/04, C22C 38/28, C22C 38/32, C21D 8/06, C21D 9/52, C21D 7/02, C22C 38/00, C22C 38/14

(54) **HIGH STRENGTH STEEL WIRE HAVING EXCELLENT CORROSION RESISTANCE AND METHOD FOR MANUFACTURING SAME**
HOCHFESTER STAHLDRAHT MIT HERVORRAGENDER KORROSIONSBESTÄNDIGKEIT UND VERFAHREN ZUR HERSTELLUNG DAVON
FIL D'ACIER À HAUTE RÉSISTANCE PRÉSENTANT UNE EXCELLENTE RÉSISTANCE À LA CORROSION ET SON PROCÉDÉ DE FABRICATION

(30) Priority: 08.12.2016 KR 20160166820
(43) Date of publication of application: 16.10.2019
(73) Proprietor: POSCO, Nam-gu Pohang-si, Gyeongsangbuk-do 37859 (KR)
(72) Inventor: LEE, Choong-Yeol, Pohang-si Gyeongsangbuk-do 37877 (KR); PARK, Yong-Sik, Pohang-si Gyeongsangbuk-do 37877 (KR)
(74) Representative: Potter Clarkson
(86) International application number: PCT/KR2017/013821
(87) International publication number: WO 2018/105944

(56) References cited:
- JP-A- H08 164 413
- JP-A- H08 164 413
- KR-A- 20160 063 534
- KR-A- 20160 063 553
- KR-A- 20160 063 553
- KR-A- 20160 063 563
- KR-A- 20160 063 565
- KR-A- 20160 075 957

## Description

### [Technical Field]

The present invention relates to a high strength steel wire, and more particularly, to a high strength steel wire having excellent corrosion resistance and a method for manufacturing the same.

### [Background Art]

An armor cable is a reinforcing material supporting the load on a flexible pipe transporting crude oil at sea, and requires high strength, as well as corrosion resistance in a corrosive environment.

A method for obtaining required physical properties in the armor cable may be as follows.

First is a method of increasing the strength of material itself by adding a large amount of elements that increase the strength of steel. A representative example of strength increasing elements of steel is carbon. As the carbon content increases, the fraction of cementite, a hard phase, increases in a wire rod, and the lamellar spacing of a pearlite structure becomes significantly small, thereby improving the strength of a material.

However, carbon is effective for improving strength, but inhibits corrosion resistance. Therefore, there is a limit to selecting an appropriate content according to a use environment.

Second is a method of drastically improving strength by drawing out a wire rod and imparting work hardening thereto. The drawing material is obtained by drawing and heat treating a rolled wire rod to be processed to form a final wire. When such a wire drawing process is carried out, the lamellar spacing becomes significantly small, the work hardening coefficient increases, and dislocations accumulate, thereby imparting work hardening.

Third, strength of a tire cord material may be improved by increasing drawing strain on the tire cord material. In this case, since the drawing strain of the material is closely related to ductility of the material, if there is no disconnection in a workpiece itself during a drawing process and the process thereof is facilitated, the material may be advantageous to improve strength.

However, since in an alloying composition, manufacturing conditions, a structure, and the like are related mutually to change the strength of a steel material, the above-described methods have limitations in improving strength by independently controlling an alloying composition, manufacturing conditions, a structure, and the like. In addition, the above methods are not considered in terms of corrosion resistance of a high strength steel wire, and thus, there is a limit to improving corrosion resistance.

KR 2016 0063553 A discloses a steel wire comprising by weight%, 0.07 to 0.15% of carbon (C), 2.7 to 3.5% of manganese (Mn), 0.10 or less of silicon (Si), 0% to 0.8% of chromium (Cr), 0.01 to 0.02% of titanium (Ti), 0.001 to 0.003% of boron (B), 0.05% or less of Nitrogen (N), 0.015% or less of Sulphur (S) and a remainder of iron (Fe) and unavoidable impurities. The microstructure of the steel wire is a mixture including bainite.

KR 2016 0063565 A also discloses a steel wire comprising by weight%, 0.07 to 0.15% of carbon (C), 2.7 to 3.5% of manganese (Mn), 0.50 to 1.50% of silicon (Si), 0% to 0.8% of chromium (Cr), 0.01 to 0.02% of titanium (Ti), 0.001 to 0.003% of boron (B), 0.05% or less of Nitrogen (N), 0.015% or less of Sulphur (S) and a remainder of iron (Fe) and unavoidable impurities. The microstructure of the steel wire is a mixture including bainite.

KR 20160075957 A also discloses a high strength, high corrosion resistance steel wire for a flexible pipe for transporting crude oil at sea and a method of manufacturing the same.

### [Disclosure]

### [Technical Problem]

The present invention is to provide a steel wire having high strength as well as high corrosion resistance even with the omission of a heat treatment, and a method for manufacturing the same.

### [Technical Solution]

The disclosed invention is defined by the appended claims.

According to an aspect of the present disclosure, a high strength steel wire having excellent corrosion resistance includes, by weight%, 0.07 to 0.15% of carbon (C), 2.7 to 3.5% of manganese (Mn), 0.10 to 0.50% of silicon (Si), 0% to 0.8% of chromium (Cr), 0.01 to 0.02% of titanium (Ti), 0.001 to 0.003% of boron (B), 0.005% or less of Nitrogen (N), 0.015% or less of Sulphur (S) and a remainder of iron (Fe) and other unavoidable impurities, wherein the microstructure of the steel wire consists of a bainite phase.

According to another aspect of the present disclosure, a method of manufacturing a high strength steel wire having excellent corrosion resistance includes producing a wire rod including, by weight%, 0.07 to 0.15% of carbon (C), 2.7 to 3.5% of manganese (Mn), 0.10 to 0.50% of silicon (Si), 0% to 0.8% of chromium (Cr), 0.01 to 0.02% of titanium (Ti), 0.001 to 0.003% of boron (B), 0.005 or less of Nitrogen (N), 0.015% or less of Sulphur (S) and a remainder of iron (Fe) and unavoidable impurities; cold-drawing the wire rod at a total reduction ratio of 40 to 80% to produce a cold drawn wire rod; and cold-rolling the cold drawn wire rod at a total reduction ratio of 50 to 90% to produce a cold rolled material, wherein the producing of the wire rod comprises preparing a billet; heating the billet at a temperature of 1000 to 1100°C; finishing wire-rolling the heated billet at a temperature of 950 to 1100°C to produce a wire rod; and cooling the wire rod at a cooling rate of 1 to 3°C/s.

### [Advantageous Effects]

According to an embodiment of the present disclosure, a steel wire having high strength, even with the omission of an LP heat treatment process, may be provided, and a steel wire according to an embodiment of the present disclosure exhibits an effect of securing excellent corrosion resistance.

Accordingly, a steel wire according to an embodiment of the present disclosure may be advantageously applicable to usage of requiring high strength and high corrosion resistance.

### [Best Mode]

The inventors have conducted in-depth research to provide a steel wire that may be suitably used in environments requiring high corrosion resistance as well as high strength. As a result, it has been found that a steel wire having a microstructure advantageous for simultaneously securing both high strength and high corrosion resistance may be provided by optimizing an alloy composition and manufacturing conditions of steel, and thus the present disclosure has been obtained.

Hereinafter, an embodiment of the present disclosure will be described in detail.

A high strength steel wire having excellent corrosion resistance according to an embodiment of the present disclosure includes, by weight%, 0.07 to 0.15% of carbon (C), 2.7 to 3.5% of manganese (Mn), 0.10 to 0.50% of silicon (Si), 0% to 0.8% of chromium (Cr), 0.01 to 0.02% of titanium (Ti), 0.001 to 0.003% of boron (B) 0.005% or less of Nitrogen (N), 0.015% or less of Sulphur (S) and a remainder of iron (Fe) and unavoidable impurities.

Hereinafter, the reason that the alloy composition of a steel wire provided in the present disclosure is controlled as described above will be described in detail. In this case, the content of respective elements refers to weight% unless otherwise specified.

### C: 0.07 to 0.15%

Carbon (C) is an element favorable for improving the strength of a steel wire. If the content of C is less than 0.07%, the strength is lowered. On the other hand, if the content of C exceeds 0.15%, the strength is improved, while ductility is decreased. In detail, corrosion resistance characteristics of the steel wire tend to decrease as the content of C increases.

In the present disclosure, the content of C is controlled to be 0.07 to 0.15% in terms of ensuring strength and corrosion resistance of the steel wire. In more detail, the content of C may be 0.09 to 0.13%.

### Mn: 2.7 to 3.5%

Manganese (Mn) is an element to secure an intended microstructure as well as improving quenching properties of a steel wire. If the content of Mn is less than 2.7%, it may be difficult to secure quenching properties, and thus, there is a problem in which a required microstructure and strength may not be obtained. On the other hand, if the content of Mn exceeds 3.5%, there is a problem in which ductility is significantly lowered.

Therefore, in the present disclosure, the content of Mn is controlled to be 2.7 to 3.5%, and, in more detail, 2.8 to 3.3%.

### Si: 0.10 to 0.50%

Silicon (Si) is an element favorable for a deoxidation effect, and Si may be added in an amount of 0.10% or more to obtain a sufficient deoxidation effect. If the content of Si is less than 0.10%, a deoxidation effect is insufficient and there is a possibility that inclusions will increase, which leads to a high possibility that ductility and corrosion resistance will be degraded. On the other hand, if the content of Si exceeds 0.50%, drawability and plate rolling properties are deteriorated.

Therefore, in the present disclosure, the content of Si is controlled to be 0.10 to 0.50%, and, in more detail, 0.15 to 0.40%.

### Cr: 0.8% or Less

Chromium (Cr) is an element favorable for securing a bainite phase as the microstructure of a steel wire by securing quenching properties, and is also an element for strength improvement.

In the present disclosure, Cr may be further included for the above-mentioned effect, but if the content exceeds 0.8%, there is a fear that a martensite phase may be formed as a microstructure, to deteriorate drawability.

Therefore, in the present disclosure, the content of Cr is controlled to be 0.8% or less when Cr is added, and even in a case in which Cr is not added, since a required microstructure and strength may be secured, 0% is included.

### Ti: 0.01 to 0.02%

Titanium (Ti) is a most reactive element with nitrogen (N), and forms nitrides in the steel. In the present disclosure, by adding Ti to form TiN, most nitrogen in the steel is exhausted, such that the formation of BN may be significantly reduced by reacting boron (B) with the N. For example, by allowing the B to exist in a soluble state, the improvement in hardenability may be obtained.

For the above-mentioned effect, Ti is added in an amount of 0.01% or more, but when the content exceeds 0.02%, a coarse nitride is formed to deteriorate mechanical properties.

Therefore, in the present disclosure, the Ti content is controlled to be 0.01 to 0.02%, and in more detail, to be 0.012 to 0.07%.

### B: 0.001 to 0.003%

Boron (B) is an element which is advantageous for improving hardenability of steel, and provides an effect of diffusing into an austenite grain boundary system to suppress formation of ferrite during cooling and increase quenching properties.

To sufficiently obtain the above-mentioned effect, B may be added in an amount of 0.001% or more. However, if the content exceeds 0.003%, not only the above effect is saturated but also boron-based nitride precipitates, deteriorating grain boundary strength and lowering hot workability.

Therefore, in the present disclosure, the content of B is controlled to be 0.001 to 0.003%.

On the other hand, as described above, an upper limit of the nitrogen (N) forming the TiN is limited to 0. 005%, such that boron (B) in steel may be maintained in a solid solution state, instead of precipitates (ex., BN), to sufficiently exhibit an effect of improving hardenability.

Further, since sulfur (S) forms low melting sulfides to deteriorate hot rolling properties and deteriorate drawing processability, an upper limit of S is limited to 0.015%.

In an embodiment of the present disclosure, the remainder is iron (Fe). However, in an ordinary manufacturing process, impurities which are not intended may be inevitably incorporated from a raw material or a surrounding environment, which cannot be excluded. These impurities are known to those skilled in the manufacturing field, and thus, are not specifically mentioned in this specification.

A steel wire according to an embodiment of the present disclosure satisfying the alloy composition described above includes a bainite single phase as a microstructure.

To secure high strength of a steel wire in an embodiment of the present disclosure, instead of forming a pearlite phase having fine lamellar spacing, a uniform bainite phase with a microstructure is formed, thereby providing a steel wire having high strength and high corrosion resistance, and simultaneously, providing a technical significance in that an existing LP heat treatment process may be omitted.

In addition to the alloy composition described above, the steel wire according to an embodiment of the present disclosure, having a bainite phase as a microstructure, has a yield strength of 1100 MPa or more and a tensile strength of 1200 MPa or more. Thus, the steel wire according to an embodiment has not only high strength but also excellent corrosion resistance in which sulfuric acid corrosion loss is 800g/mm²·h or lower.

Hereinafter, a method of manufacturing a high strength steel wire having excellent corrosion resistance, according to another embodiment in the present disclosure, will be described in detail.

A steel wire according to an embodiment in the present disclosure may be produced by a process of manufacturing a wire rod satisfying the above-described alloy composition, and then, of drawing the wire rod.

Although the wire rod may be manufactured through a variety of wire rod manufacturing techniques known in the art, in detail, the wire rod may be manufactured through a series of processes to be described below.

First, a billet satisfying the above-mentioned alloy composition is manufactured, and may then be subjected to a heating process of homogenizing the billet.

A microstructure of the billet may be formed as an austenite single phase through the heating process.

To this end, the heating is performed in a temperature range of 1000 to 1100°C. If the heating temperature is less than 1000°C, it may be difficult to secure a temperature region in subsequent wire rolling. If the heating temperature exceeds 1100°C, austenite grains are formed coarsely and a target level of strength may be difficult to secure.

The billet heated as described above is subjected to wire rolling, and then, is cooled to be produced as a wire rod.

In this case, as the wire rolling, finishing hot rolling is performed in a temperature range of 950 to 1100°C. If a temperature during the finishing hot rolling is less than 950°C, there is a problem in which roll life is reduced due to an increase in a rolling load. On the other hand, if the temperature exceeds 1100°C, the grain size becomes coarse, and thus, ductility may be reduced. Further, in this case, decarburization may occur excessively, thereby deteriorating drawability.

Thereafter, a wire rod having a bainite phase is manufactured by cooling at a cooling rate of 1 to 3°C/s. If the cooling rate is less than 1°C/s, there is a fear that a structure such as pearlite or the like, other than the bainite phase, may be formed as a microstructure, while if the cooling rate exceeds 3°C/s, there is a fear that a martensite phase may be formed.

A steel wire is manufactured by drawing the wire rod manufactured as described above. In the present disclosure, descriptions of an LP heat treatment generally performed before the wire rod is drawn will be omitted.

According to an embodiment in the present disclosure, since the wire rod having a uniform bainite phase, without a ferrite structure, is subjected to a drawing process, homogeneity and a relatively high work-hardening ratio may be secured without performing a separate LP heat treatment.

In more detail, the wire rod may be directly cold-drawn without a LP heat treatment process, and in this case, a cold drawn wire rod is manufactured by performing cold drawing on the wire rod at a reduction ratio of 40 to 80% in total.

If the reduction ratio is less than 40% in cold drawing, since the amount of drawing processing is insufficient, sufficient strength may not be secured. On the other hand, if the reduction ratio exceeds 80%, cracks may occur.

The cold drawn wire rod as described above may have a yield strength of 1000 MPa or more and a tensile strength of 1100 MPa or more.

Subsequently, the cold drawn wire rod is cold rolled, and in this case, a cold rolled material is produced by cold rolling at a total reduction ratio of 50 to 90%.

The cold rolling is to obtain a steel wire having a plate-like shape. If the reduction ratio in this case is less than 50%, a processing amount is insufficient and sufficient strength may not be ensured. On the other hand, if the reduction ratio exceeds 90%, cracks may occur.

The cold-rolled material as described above may have a yield strength of 1100 MPa or more and a tensile strength of 1200 MPa or more.

Hereinafter, embodiments in the present disclosure will be described in further detail by way of example . It should be noted, however, that the following embodiments are intended to illustrate the present disclosure in more detail and not to limit the scope of the present disclosure. The scope of the present disclosure is determined by the matters set forth in the claims and the matters reasonably inferred therefrom.

### [Mode for Invention]

### (Embodiment)

A billet having an alloy composition shown in the following Table 1 was prepared, and then, the billet was heated at 1000 to 1100°C and then hot-rolled at 1000°C to produce a wire rod. Thereafter, the wire rod was cooled to 500°C at a cooling rate of 1 to 3°C/s, followed by air-cooling to room temperature.

Then, Inventive Steels 1 to 6, which satisfy an alloy composition proposed in the present disclosure, were cold rolled at a total reduction ratio of 50 to 90%, after performing drawing at a total reduction ratio of 40 to 80%, thereby producing a steel wire. Comparative Steels 1 to 4 were subjected to an LP heat treatment and then subjected to a drawing process (a total reduction ratio of 40 to 80%) and cold rolling (a total reduction ratio of 50 to 90%).

Tensile properties of respective wire rods and steel wires fabricated above were evaluated by a room temperature tensile test. Corrosion loss of the respective steel wires was measured by immersing a steel wire in 5% sulfuric acid solution. The results are shown in Table 2 below.

**[Table 1]**

| Classific ation | Alloy Composition (Weight%) | | | | | | | |
|---|---|---|---|---|---|---|---|---|
| | C | Si | Mn | Cr | S | Ti | B | N |
| Inventive Steel 1 | 0.11 | 0.15 | 3.0 | - | 0.004 | 0.015 | 0.002 | 0.004 |
| Inventive Steel 2 | 0.11 | 0.15 | 3.0 | 0.5 | 0.004 | 0.015 | 0.002 | 0.004 |
| Inventive Steel 3 | 0.12 | 0.16 | 3.1 | - | 0.004 | 0.016 | 0.002 | 0.004 |
| Inventive Steel 4 | 0.13 | 0.13 | 3.3 | - | 0.003 | 0.012 | 0.002 | 0.004 |
| Inventive Steel 5 | 0.10 | 0.16 | 2.8 | 0.6 | 0.004 | 0.013 | 0.002 | 0.003 |
| Inventive Steel 6 | 0.10 | 0.14 | 2.7 | 0.4 | 0.003 | 0.017 | 0.002 | 0.005 |
| Comparati ve Steel 1 | 0.35 | 0.20 | 0.7 | - | 0.004 | - | - | 0.006 |
| Comparati ve Steel 2 | 0.32 | 0.24 | 0.8 | - | 0.005 | - | - | 0.007 |
| Comparati ve Steel 3 | 0.38 | 0.17 | 0.6 | - | 0.005 | - | - | 0.006 |
| Comparati ve Steel 4 | 0.33 | 0.18 | 1.3 | - | 0.011 | 0.03 | 0.07 | 0.008 |

**[Table 2]**

| Classification | LP Heat Treatment | Wire Rod | | LP Material | | Cold Rolling Wire (Steel Wire) | | Corrosi on Loss (g/mm²· h) |
|---|---|---|---|---|---|---|---|---|
| | | YS | TS | YS | TS | YS | TS | |
| Inventive Steel 1 | Not Performed | 480 | 757 | - | - | 1230 | 1331 | 527 |
| Inventive Steel 2 | Not Performed | 584 | 895 | - | - | 1344 | 1474 | 539 |
| Inventive Steel 3 | Not Performed | 483 | 762 | - | - | 1241 | 1332 | 532 |
| Inventive Steel 4 | Not Performed | 479 | 761 | - | - | 1232 | 1342 | 518 |
| Inventive Steel 5 | Not Performed | 596 | 901 | - | - | 1349 | 1489 | 548 |
| Inventive Steel 6 | Not Performed | 573 | 881 | - | - | 1330 | 1463 | 532 |
| Comparativ e Steel 1 | Performed | 293 | 327 | 451 | 687 | 1090 | 1187 | 1093 |
| Comparativ e Steel 2 | Performed | 287 | 319 | 448 | 673 | 1073 | 1163 | 1087 |
| Comparativ e Steel 3 | Performed | 312 | 334 | 467 | 692 | 1118 | 1203 | 1218 |
| Comparativ e Steel 4 | Performed | 332 | 347 | 505 | 714 | 1147 | 1198 | 1196 |

(In Table 2, YS refers to yield strength, TS refers to tensile strength, and the unit is MPa.)

As shown in Tables 1 and 2, it can be confirmed that in 5 the case of Inventive Steels 1 to 6 satisfying alloy compositions according to an embodiment of the present disclosure, strength of wire rods (yield strength and tensile strength) is improved in comparison with Comparative Steels 1 to 4. In addition, it can be confirmed that the strength of steel wires of Inventive Steels 1 to 6 is also higher than that of Comparative Steels 1 to 4 subjected to an LP heat treatment.

In other words, in the case of Inventive Steels 1 to 6 having a bainite phase as a microstructure, a work hardening rate is relatively high, and thus, required high strength may be obtained through a drawing process and cold rolling without performing an LP heat treatment, as compared with Comparative Steels 1 to 4 having a pearlite phase.

In addition, Inventive Steels 1 to 6 exhibited a corrosion loss of 550g/mm² ·h or lower, which indicates that a corrosion rate was reduced by about 50% under the same conditions as Comparative Steels 1 to 4.

As a result, the corrosion resistance may be improved by removing a ferrite phase which adversely affects corrosion resistance characteristics of a steel wire and forming a bainite phase.

## Claims

1. A high strength steel wire having excellent corrosion resistance, comprising:
by weight%, 0.07 to 0.15% of carbon (C), 2.7 to 3.5% of manganese (Mn), 0.10 to 0.50% of silicon (Si), 0% to 0.8% of chromium (Cr), 0.01 to 0.02% of titanium (Ti), 0.001 to 0.003% of boron (B), 0.005% or less of Nitrogen (N), 0.015% or less of Sulphur (S) and a remainder of iron (Fe) and unavoidable impurities,
wherein the microstructure of the steel wire consists of a bainite phase.

2. The high strength steel wire having excellent corrosion resistance of claim 1, wherein the steel wire has a sulfuric acid corrosion loss of 800g/mm²·h or less in 5% sulfuric acid solution.

3. The high strength steel wire having excellent corrosion resistance of claim 1, wherein the steel wire has a yield strength of 1100 MPa or more and a tensile strength of 1200 MPa or more.

4. A method of manufacturing a high strength steel wire having excellent corrosion resistance, the method comprising:
producing a wire rod including, by weight%, 0.07 to 0.15% of carbon (C), 2.7 to 3 .5% of manganese (Mn), 0.10 to 0.50% of silicon (Si), 0% to 0.8% of chromium (Cr), 0.01 to 0.02% of titanium (Ti), 0.001 to 0.003% of boron (B), 0.005% or less of Nitrogen (N), 0.015% or less of Sulphur (S) and a remainder of iron (Fe) and unavoidable impurities;
cold-drawing the wire rod at a total reduction ratio of 40 to 80% to produce a cold drawn wire rod; and
cold-rolling the cold drawn wire rod at a total reduction ratio of 50 to 90% to produce a cold rolled material, wherein the producing of the wire rod comprises preparing a billet; heating the billet at a temperature of 1000 to 1100°C; finishing wire-rolling the heated billet at a temperature of 950 to 1100°C to produce a wire rod; and cooling the wire rod at a cooling rate of 1 to 3°C/s.

5. The method of manufacturing a high strength steel wire having excellent corrosion resistance of claim 4, wherein the cold drawn wire rod has a yield strength of 1000 MPa or more and a tensile strength of 1100 MPa or more.

6. The method of manufacturing a high strength steel wire having excellent corrosion resistance of claim 4, wherein the cold rolled material has a yield strength of 1100 MPa or more and a tensile strength of 1200 MPa or more.

## Patentansprüche

1. Hochfester Stahldraht mit ausgezeichneter Korrosionsbeständigkeit, umfassend:
in Gewichts-% 0,07 bis 0,15 % Kohlenstoff (C), 2,7 bis 3,5 % Mangan (Mn), 0,10 bis 0,50 % Silicium (Si), 0 bis 0,8 % Chrom (Cr), 0,01 bis 0,02 % Titan (Ti), 0,001 bis 0,003 % Bor (B), 0,005 % oder weniger Stickstoff (N), 0,015 % oder weniger Schwefel (S) und ein Rest Eisen (Fe) und unvermeidbare Verunreinigungen,
wobei die Mikrostruktur des Stahldrahts aus einer Bainitphase besteht.

2. Hochfester Stahldraht mit ausgezeichneter Korrosionsbeständigkeit nach Anspruch 1, wobei der Stahldraht einen Schwefelsäurekorrosionsverlust von 800 g/mm²/h oder weniger in 5 % Schwefelsäurelösung aufweist.

3. Hochfester Stahldraht mit ausgezeichneter Korrosionsbeständigkeit nach Anspruch 1, wobei der Stahldraht eine Streckgrenze von 1100 MPa oder mehr und eine Zugfestigkeit von 1200 MPa oder mehr aufweist.

4. Verfahren zur Herstellung eines hochfesten Stahldrahtes mit ausgezeichneter Korrosionsbeständigkeit, wobei das Verfahren umfasst:
Herstellung eines Walzdrahtes, der in Gewichts-% 0,07 bis 0,15 % Kohlenstoff (C), 2,7 bis 3,5 % Mangan (Mn), 0,10 bis 0,50 % Silicium (Si), 0 bis 0,8 % Chrom (Cr), 0,01 bis 0,02 % Titan (Ti), 0,001 bis 0,003 % Bor (B), 0,005 % oder weniger Stickstoff (N), 0,015 % oder weniger Schwefel (S) und ein Rest Eisen (Fe) und unvermeidbare Verunreinigungen einschließt;
Kaltziehen des Walzdrahtes mit einem Gesamtreduzierungsverhältnis von 40 bis 80 %, um einen kaltgezogenen Walzdraht herzustellen; und
Kaltwalzen des kaltgezogenen Walzdrahtes mit einem Gesamtreduzierungsverhältnis von 50 bis 90 %, um ein kaltgewalztes Material herzustellen, wobei das Herstellen des Walzdrahtes das Vorbereiten eines Knüppels umfasst;
Erhitzen des Knüppels auf eine Temperatur von 1000 bis 1100 °C;
Fertigstellen des Drahtwalzens des erhitzten Knüppels bei einer Temperatur von 950 bis 1100 °C, um einen Walzdraht herzustellen; und
Abkühlen des Walzdrahtes mit einer Abkühlgeschwindigkeit von 1 bis 3 °C/s.

5. Verfahren zur Herstellung eines hochfesten Stahldrahtes mit ausgezeichneter Korrosionsbeständigkeit nach Anspruch 4, wobei der kaltgezogene Walzdraht eine Streckgrenze von 1000 MPa oder mehr und eine Zugfestigkeit von 1100 MPa oder mehr aufweist.

6. Verfahren zur Herstellung eines hochfesten Stahldrahtes mit ausgezeichneter Korrosionsbeständigkeit nach Anspruch 4, wobei das kaltgewalzte Material eine Streckgrenze von 1100 MPa oder mehr und eine Zugfestigkeit von 1200 MPa oder mehr aufweist.

## Revendications

1. Fil d'acier à haute résistance ayant une excellente résistance à la corrosion, comprenant :
en % en poids, 0,07 à 0,15 % de carbone (C), 2,7 à 3,5 % de manganèse (Mn), 0,10 à 0,50 % de silicium (Si), 0 % à 0,8 % de chrome (Cr), 0,01 à 0,02 % de titane (Ti), 0,001 à 0,003 % de bore (B), 0,005 % ou moins d'azote (N), 0,015 % ou moins de soufre (S) et un reste de fer (Fe) et des impuretés inévitables,
la microstructure du fil d'acier étant constituée d'une phase bainite.

2. Fil d'acier à haute résistance ayant une excellente résistance à la corrosion selon la revendication 1, dans lequel le fil d'acier a une perte par corrosion d'acide sulfurique de 800 g/mm²•h ou moins dans une solution d'acide sulfurique à 5 %.

3. Fil d'acier à haute résistance ayant une excellente résistance à la corrosion selon la revendication 1, dans lequel le fil d'acier a une limite d'élasticité de 1 100 MPa ou plus et une résistance à la traction de 1 200 MPa ou plus.

4. Procédé de fabrication d'un fil d'acier à haute résistance ayant une excellente résistance à la corrosion, le procédé comprenant :
la production d'un fil machine comportant, en % en poids, 0,07 à 0,15 % de carbone (C), 2,7 à 3,5 % de manganèse (Mn), 0,10 à 0,50 % de silicium (Si), 0 % à 0,8 % de chrome (Cr), 0,01 à 0,02 % de titane (Ti), 0,001 à 0,003 % de bore (B), 0,005 % ou moins d'azote (N), 0,015 % ou moins de soufre (S) et un reste de fer (Fe) et des impuretés inévitables ;
l'étirage à froid du fil machine à un rapport de réduction total de 40 à 80 % pour produire un fil machine étiré à froid ; et
le laminage à froid du fil machine étiré à froid à un rapport de réduction total de 50 à 90 % pour produire un matériau laminé à froid, dans lequel la production du fil machine comprend la préparation d'une billette ; le chauffage de la billette à une température de 1 000 à 1 100 °C ; la finition du laminage de fil de la billette chauffée à une température de 950 à 1 100 ° C pour produire un fil machine ; et le refroidissement du fil machine à une vitesse de refroidissement de 1 à 3 °C/s.

5. Procédé de fabrication d'un fil d'acier à haute résistance ayant une excellente résistance à la corrosion selon la revendication 4, dans lequel le fil machine étiré à froid a une limite d'élasticité de 1 000 MPa ou plus et une résistance à la traction de 1 100 MPa ou plus.

6. Procédé de fabrication d'un fil d'acier à haute résistance ayant une excellente résistance à la corrosion selon la revendication 4, dans lequel le matériau laminé à froid a une limite d'élasticité de 1 100 MPa ou plus et une résistance à la traction de 1 200 MPa ou plus.
